

May 27, 1941.

J. F. OLIN

2,243,471

## MANUFACTURE OF NITRIC ACID ESTERS

Filed Nov. 15, 1938



## UNITED STATES PATENT OFFICE

2,243,471

## MANUFACTURE OF NITRIC ACID ESTERS

John F. Olin, Grosse Ile, Mich., assignor to The  
Sharples Solvents Corporation, Philadelphia,  
Pa.

Application November 15, 1938, Serial No. 240,513

20 Claims. (Cl. 260—467)

This invention relates to a process for the preparation of nitrate esters from aliphatic alcohols. The nitration of aliphatic alcohols to obtain esters of nitric acid has long presented a problem of considerable commercial importance. The potential importance of such esters is very great since they are useful as intermediates in the preparation of a wide variety of organic chemicals in addition to possessing properties that render them suitable for many purposes as ultimate products.

Heretofore, the development of uses for compounds of the alkyl nitrate type has been hampered by the lack of a process for producing such materials on a commercial scale at a reasonable price. Under prior art practice the yields of nitrated products, with very few exceptions, are low and the operations are dangerous.

Two procedures for the preparation of nitrates from methyl, ethyl, propyl, butyl and amyl alcohols have been described. One method, which has been used to prepare nitrates from monohydric alcohols containing not more than three carbon atoms, consists essentially in the distillation of a mixture of nitric acid and alcohol in the presence of urea. The nitrate formed is readily volatilized and may be distilled from the reaction zone to prevent accumulation of the ester in the nitrating vessel which might otherwise result in explosions. Since the presence of even small amounts of nitrous acid tends to initiate a vigorous auto-oxidation of explosive violence, urea is added to decompose nitrous acid as formed in accordance with the following equation:



By the above process the methyl and ethyl nitrates may be prepared with fairly good results, but the method is not suitable for the nitration of alcohols containing four or more carbon atoms. In the case of the nitration of propyl or butyl alcohol or alcohols of higher carbon content than butyl alcohol, higher temperatures are required to obtain the esterification reaction than when the lower alcohols are nitrated. Higher temperatures are also required for distillation of the esters from the nitration mixture in the case of higher alcohols than in the case of the lower alcohols. As the result of these two facts, attempts to nitrate propyl and higher alcohols have resulted in the oxidation of the alcohol to produce the corresponding aldehyde, this oxidation reaction occurring incident to nitration of the alcohol and therefore preventing the success-

ful practice of the nitration process. In such cases the oxidation of the alcohol can be to some extent prevented by the addition of urea to the reaction mixture, but even when this precaution is taken the yield of the desired nitrate is still very low. In the course of the oxidation reaction occurring when attempts are made to nitrate the higher alcohols, the nitric acid intended for esterification is reduced to nitrous acid. The oxidation of the alcohol is therefore a deleterious reaction both from the standpoint of producing undesired by-products and from the standpoint of reducing the esterifying acid. Even with the lowest alcohols the yield is rarely 15 in excess of 75% ("Systematic Organic Chemistry," Cumming, Hopper and Wheeler, page 254). A process of nitrating isoamyl alcohol which has been successful from a laboratory viewpoint involves the addition of isoamyl alcohol or a mixture of the alcohol with concentrated sulfuric acid to an ice-cold bath of nitric and concentrated sulfuric acid in the volume ratio of 1:3. This process has not achieved commercial success because of the difficulties of recovering unused nitric acid and of reconcentrating the sulfuric acid. A more serious defect of this method lies in the frequent explosions occurring unless the alcohol is very pure.

Neither of the above processes gives satisfactory results in the nitration of monohydric alcohols other than primary alcohols and no satisfactory method has been heretofore devised for the preparation of secondary alkyl nitrates. The yields obtained by treating a secondary or tertiary aliphatic alcohol by either of the methods described above are negligible. Further, it has been found that the first of these methods is unsuitable for the treatment of alcohols higher than ethyl.

It has been found that the use of dilute nitric acid avoids the objections to prior processes to some extent. Again, using amyl alcohol as an example, it was found that moderate conversion of alcohol to nitrate was obtained by treatment with 35% to 60% nitric acid. Concentrations below 30% gave very low-grade esters while the use of acid having a nitric acid content in excess of 50% resulted in substantial oxidation with consequent decrease in yield. The present invention rests upon a procedure by which the objectionable features of prior art processes are avoided by passing the reactants to the reaction chamber in a continuous manner and continuously passing the reaction mixture from the reaction chamber, this mixture being separated

into its constituents only after it has been removed from the reaction chamber. By adopting this procedure and the other features of the invention discussed hereinafter, the proportions of the respective constituents of the reaction mixture in the esterification vessel are maintained substantially constant.

An object of this invention has been the provision of a process for reacting an aliphatic alcohol with nitric acid to produce a commercially practicable yield of ester, and a most important object has been to afford a satisfactory method of producing nitrates of propyl and higher alcohols. The practice of the features of the invention is particularly useful in producing alkyl nitrates by esterifying alcohols containing from 3 to 8 carbon atoms, inclusive, with nitric acid.

It may be logically inferred that the esterification of an aliphatic alcohol proceeds through the formation of an oxonium derivative of very low vapor pressure. From that intermediate compound, the ester is formed by loss of water, but in the presence of concentrated nitric acid, the oxonium derivative is oxidized to form undesired by-products. These reactions may be represented as follows:



In the above equations the reactions represented by Equations 1 and 2 are the desirable reactions, while the reaction represented by Equation 3 is the undesirable reaction, since it results in the formation of undesired valeraldehyde and reduction of the nitric acid which might otherwise be converted into amyl nitrate.

When concentrated nitric acid is used in the practice of the process of nitration as indicated by Equations 1 to 3 above, the reactions of Equations 1 and 3 predominate, and the desired reaction of Equation 2 is depressed.

When concentrated nitric acid is used, the concentrated nitric acid also causes auto-oxidation of the alkyl nitrate formed in accordance with Equation 2 above, with the result that the contents of the reaction vessel frequently explode.

On the other hand, when very dilute nitric acid is employed in this reaction, the reaction is extremely slow and the yields of the desired products are small.

The operator, desiring to produce amyl nitrate, for example, is on the horns of a dilemma when attempting to operate in accordance with the prior art procedure for producing methyl and ethyl nitrates. If he initiates the reaction with the use of a concentrated nitric acid, the initial reaction involves undesired production of valeraldehyde and reduction of the nitric acid as indicated in Equation 3. If, on the other hand, he initiates the reaction by the use of nitric acid of the concentration found most suitable for the accomplishment of the reactions of Equations 1 and 2, water formed incident to the esterification reaction as indicated in Equation 2 rapidly dilutes the reaction mixture and reduces the nitric acid to a concentration at which it will not efficiently perform its nitrating function.

Reasoning from the above premises, the ap-

plicant conceived the present invention and solved the difficulties of the prior art procedures by developing nitration technique whereby the concentration of the nitric acid in the esterification vessel is maintained substantially constant, and may be maintained at such point as to effectively accomplish the nitration function while minimizing the occurrence of the undesired reaction of Equation 3, and minimizing the occurrence of auto-oxidation of the alkyl nitrate formed in accordance with Equation 2.

In accordance with the present invention, auto-oxidation in the esterification vessel is prevented by removing the alkyl nitrate from the esterification vessel promptly after the formation thereof. This is accomplished by passing the reactants continuously through the reaction apparatus, nitric acid, the alcohol to be esterified and an amount of urea sufficient to inhibit auto-oxidation being continuously passed to the reaction vessel and a mixture of alkyl nitrate, alcohol, nitric acid and water being continuously discharged from the esterification vessel. By proceeding in this manner, the concentration of nitric acid in the esterification vessel may be maintained substantially constant, since the water of esterification is removed from that vessel at the same rate at which it is formed incident to the esterification. The reaction mixture is thereafter separated into its constituents by extraction and distillation steps to be described hereinafter.

Since there is usually a tendency toward formation of nitrous acid in the reaction mass which will initiate oxidation if permitted to accumulate, it is preferred that a small proportion of urea be added to the vessel in which the present process is practiced. As a general rule the proportion of urea added is less than that employed in the process of the prior art, but as a precaution against decreased yields, inferior grade ester, and explosion it is always well to follow the practice of adding at least a small amount of urea.

In its preferred embodiment the invention may be advantageously practiced in the apparatus shown diagrammatically in the accompanying drawing wherein 10, 11 and 12 designate storage tanks which may contain nitric acid of the desired concentration, an alcohol and 50% urea solution respectively, and each of these tanks is connected by a valved pipe to reaction vessel 13, which is provided with an agitator and a heating coil.

In the practice of the invention, nitric acid is first passed into the reaction vessel 13 to a level slightly below the level of the takeoff line which connects that vessel with the mixer 14. A small quantity of urea is also preferably passed to the reaction vessel 13 at this time. The nitric acid is then heated to the desired temperature at which it is reacted with the alcohol to be esterified. Quantities of alcohol from tank 11 and an excess of nitric acid from tank 10 are then run continuously into the esterification vessel 13. Since the temperature in the reaction vessel 13 is at the point best facilitating the reaction, the alcohol and nitric acid will react promptly upon contact with each other in that vessel. The reaction mixture, containing the desired alkyl nitrate, unreacted nitric acid, water of esterification, urea and alcohol, passes continuously from the esterification vessel 13 to a mixer 14, which is provided with a mechanical agitator.

The rate of withdrawal of the reaction mixture from the esterification vessel 13 to the mixer

14 is substantially the same as the rate of passage of nitric acid and alcohol from containers 10 and 11 to the esterification vessel. A solvent for the ester content of the reaction mixture is continuously passed from tank 15 to mixer 14 in such proportion as to selectively dissolve the ester and alcohol in the mixer 14 to the substantial exclusion of nitric acid and water. The solvent added in mixer 14 may be any good, inert, oil solvent, such as benzene, toluene, hexane, heptane, ether or a chlorinated hydrocarbon solvent such as carbon tetrachloride. In case the ester formed is heavier than the nitric acid solution contained in the mixture passed to the mixer 14, it is preferable to employ a solvent of high specific gravity, such as carbon tetrachloride, in order to facilitate subsequent separation of the solution of ester and alcohol in the solvent from the nitric acid of the reaction mixture. In cases in which, on the other hand, the ester formed is lighter than the nitric acid solution passed to the mixer 14, it is preferred to employ a solvent of lower specific gravity than that of the nitric acid solution, such as benzene, toluene, hexane, heptane or ether. The mixer 14 is preferably provided with a coil, through which a cooling liquid is circulated in order to prevent volatilization in case a high volatile solvent, such as ether, is employed.

The mixture of nitric acid solution and solution of ester and alcohol in the solvent is next passed to a decanter 16, in which the major part of the nitric acid solution is removed from the solution of ester and alcohol in the solvent from tank 15. The nitric acid solution may be passed to receiver 17 for subsequent fractionation to remove organic constituents and reconcentration. The solution of ester and alcohol in the solvent is passed from decanter 16 to a mixer 18. It is to be noted at this point that, if the nitric acid solution is of lower specific gravity than the ester solution (oil layer) decanted from decanter 16, the decanter connections will be reversed, the lighter effluent (nitric acid solution) being passed to receiver 17 and the heavier effluent to receiver 18.

Water from tank 19' is mixed with the oil layer passing to tank 18 from decanter 16, and the mixture so produced is passed continuously to a decanter 18, where the aqueous layer is removed and sent to the receiver 17. The oil layer from decanter 19 (which may be the lighter or heavier layer, depending upon the specific gravity of the ester produced and the specific gravity of the solvent used) is passed continuously to a mixer 20, where it is treated with an aqueous alkaline solution, such as a sodium carbonate solution, which removes the last traces of free acid. This alkaline solution is passed from tank 22 to the mixer 20 and the mixture produced in the mixer 20 is then passed to a decanter 21, which effects removal from the oily solution of the alkaline aqueous liquid produced in mixer 20. The aqueous alkaline solution is passed to receiver 23 and the oil layer from decanter 21 is passed to a mixer 24, where it is again mixed with water from container 19. The mixture from mixer 24 is passed to a decanter 25, from which the aqueous layer is passed to receiver 23, while the oil layer is passed to stripping apparatus to be described hereinafter.

The material collected in the receiver 23, like the material collected in receiver 17, is subjected to a stripping operation to remove unused alcohol, and this unused alcohol may be returned

5 to the tank 11. The oil layer from decanter 25 is next passed to a stripping column 26, which is maintained at such a temperature that the solvent passes overhead and is condensed in condenser 27 and returned to the tank 15. A residue consisting of unused alcohol and the nitric acid ester collects in the still 28, and this residue is pumped into column 29, which is operated at such a temperature as to pass the alcohol overhead in the form of a binary constant boiling mixture containing a part of the alkyl nitrate. This overhead fraction is condensed in condenser 30. A part of the condensate is refluxed to column 29 and another part may be returned to tank 11 as illustrated.

10 After separation of the alcohol content of this mixture from the desired nitrate, this alcohol may be returned to storage tank 11. Alkyl nitrate is pumped from the still 31 into a column 32, where further purification of this ester is obtained, followed by condensation in the condenser 34. The ester so obtained from condenser 34 is sufficiently pure to be used commercially. In cases in which relatively high boiling esters 15 are produced, it is preferable to maintain the columns 26, 29 and 32 under sub-atmospheric pressure in order to avoid decomposition of these esters, which might occur in case the temperatures necessary to effect distillation at atmospheric pressure were employed.

20 The use of concentrated acid, that is, nitric acid containing substantially more than 70% HNO<sub>3</sub>, is possible under very closely controlled conditions, but should be avoided in most nitration reactions of the present type. The term "dilute nitric acid" as used in this disclosure and in the claims appended hereto is to be understood as referring to an acid containing HNO<sub>3</sub> not substantially in excess of 70%. It has been noted that extremely dilute acids generally give slow reactions and poor conversions and although some of the benefits of this invention may be obtained with acid of low concentration it is usually found that better results are obtained when using nitric acid having an HNO<sub>3</sub> content in excess of 30%; i. e., in which the total water content of the esterification vessel does not bear a ratio to the total HNO<sub>3</sub> content of greater than 70:30. While acids having a concentration between about 30% and 65% give highly satisfactory results as compared with prior processes, the preferred range is 45% to 55% concentration of nitric acid since a reagent within the latter limits has been found generally suitable to the nitration of alcohols esterified in accordance with the present invention. The acid added continuously to the esterification vessel should be of somewhat higher concentration than the concentration of acid which it is desired to maintain in that vessel, since acid continuously added to the vessel will be diluted to the desired concentration by the water of esterification formed in that vessel. A fairly good general rule is that lower acid concentrations should be used in connection with alcohols having a greater number of substituents on the carbinol group, e. g., that lower acid concentrations should be used in esterifying secondary alcohols than primary alcohols.

25 The use of urea is recommended to inhibit oxidation. The process here described represents a striking improvement over the prior art by depressing side reactions to the very minimum and the amount of urea required is therefore very small. The low cost of this reagent in the

amounts used in the preferred embodiment of this invention is fully justified by the additional safety and improved yield obtained thereby. In connection with the nitration of primary alcohols, such as butanol-1, very little of the oxidation inhibitor is normally used, while more highly substituted carbinols generally require appreciable amounts of this reagent.

*Example 1—Preparation of normal propyl nitrate.*—Reaction vessel 13 is charged with 60% nitric acid and a 50% solution of urea in water is added from tank 12 in an amount constituting 5% of the weight of nitric acid in the esterification vessel 13. Steam is then passed into the heating coil of the vessel 13 until the contents are raised to a temperature between 80 and 85° C. The agitator in the vessel 13 is then started and further quantities of 70% nitric acid from tank 10 and normal propyl alcohol from tank 11 are run in, in approximate volume ratio of 1.3 to 1. As the reaction proceeds, further quantities of urea solution in amounts necessary to inhibit oxidation are added. Simultaneously with the addition of acid, alcohol and urea liquid overflows from esterification vessel 13 into mixer 14, and the mixture in mixer 14 is reduced to a temperature of 25° C. An amount of normal hexane equal in volume to the volume of alcohol passed from tank 11 to vessel 13, is continuously supplied to the mixer 14. The mixture passing from mixer 14 is decanted in decanter 16 and the oil layer from decanter 16 is further washed and decanted, as indicated in the above description. The washed ester from decanter 25 is then passed into column 26, where the hexane containing traces of propyl alcohol and propyl nitrate is passed overhead and returned to storage tank 15. The bottoms from still 28 are then pumped into column 29, and the small amount of propyl alcohol remaining in the crude mixture is passed overhead, together with some propyl nitrate, and returned to storage tank 11. The crude ester is then rectified by pumping it from still 31 into column 32 and obtaining relatively pure propyl nitrate boiling between 108 and 111° C. The ester produced in this manner has a specific gravity of 1.045.

In the case of the preparation of this ester, it is to be observed that, because of the solubility of propyl alcohol in the diluted nitric acid and in the aqueous wash water passed to receivers 17 and 23, only a relatively small quantity of propyl alcohol was recovered in the subsequent distillation operations performed in columns 26 and 29. However, upon distilling the diluted acid from receiver 17 and the diluted alkaline washes from receiver 23, substantially all of the propyl alcohol not accounted for as propyl nitrate may be recovered.

*Example 2—Mixed amyl nitrates.*—In the manufacture of this material, 50% nitric acid is charged into vessel 13 to approximately a point one-third below the takeoff. Upon heating to 90° C., esterification is caused to take place by the continuous addition of amyl alcohol and 65% nitric acid; the latter being used in 50% excess, or such excess as is required to maintain the free acid at 40-50%. Benzene may be used as a solvent instead of hexane, if desired, and the absolute pressure in the fractionation columns 26, 29 and 32 is preferably reduced to 200 mm. The process is otherwise identical with that described in Example 1. The mixed amyl nitrate material obtained by conducting the process in this manner in the esterification with the mixture of amyl

alcohol, commercially known as Pentasol, has a specific gravity at a temperature of 20° C. of 0.988, and boils between 142 and 154.2° C. This mixture is a colorless liquid and has a pleasant odor.

From the above discussion, the manner in which the objects of the invention have been attained will be apparent. By conducting the reaction continuously, and removing the reaction mixture from the esterification vessel as formed, conditions in the esterification vessel are maintained substantially constant, and may be maintained at the point found most suitable for esterification of the particular alcohol being reacted with nitric acid. By operating in this manner, the disadvantage inherent in operating in accordance with prior art procedure of progressive dilution of the nitric acid is avoided. In view of this fact, it is not necessary to initiate the practice of the process by the use of acid of higher concentration than that most satisfactory for the preparation of the desired ester, and all of the disadvantages of the prior art discussed above are thus obviated.

While specific apparatus has been described in the foregoing description of the invention, I wish it understood that the invention is in no way limited to such specific apparatus, but that it may be practiced in any apparatus suitable for the performance of the above-described process steps. Thus, for example, the esterification vessel 13 does not necessarily have to be a reaction vessel of the type illustrated, but may be any suitable column, coil, or other contacting device, in which nitric acid of the desired strength is brought into contact with alcohol, and from which the reaction mixture is continuously discharged to apparatus for the performance of a series of steps in which the reaction mixture is separated into its constituents, as described.

Still further modifications will be obvious to those skilled in the art and I do not therefore wish to be limited except by the scope of the subjoined claims.

I claim:

1. The process of preparing an aliphatic nitrate which comprises continuously passing nitric acid of between forty-five and fifty-five percent concentration and an aliphatic alcohol together through a reaction zone, continuously removing the reaction mixture from said reaction zone during the feed of nitric acid and alcohol thereto, and thereafter separating the desired aliphatic nitrate from the reaction mixture so produced by solvent extraction.

2. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate.

3. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent chosen from the class consisting of chlorin-

ated hydrocarbons, benzene, toluene, hexane, heptane and ether.

4. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate and subsequent washing with water of the material dissolved in the extraction solvent.

5. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate, washing with water the material dissolved in the extraction solvent and subsequently neutralizing the water-washed mixture by washing with a base.

6. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate, washing with water the material dissolved in the extraction solvent, neutralizing the water-washed mixture by washing with a base and thereafter again washing the solvent-extracted, water-washed and neutralized mixture with water.

7. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate and subsequent distillation of the extracted organic constituents of the reaction mixture to separate solvent and alcohol therefrom.

8. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate, washing with water the material dissolved in the extraction solvent and subsequent distillation of the extracted organic constituents of the reaction mixture to separate solvent and alcohol therefrom.

9. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter 75

separating the desired aliphatic nitrate from the reaction mixture so produced by a process involving extraction of the reaction mixture with a solvent for said aliphatic nitrate, washing with water the material dissolved in the extraction solvent, neutralizing the water-washed mixture and subsequent distillation of the extracted organic constituents of the reaction mixture to separate solvent and alcohol therefrom.

10 10. The process of preparing an aliphatic nitrate which comprises continuously passing nitric acid and an aliphatic alcohol together through a reaction zone, continuously removing the reaction mixture from said reaction zone  
15 during the feed of nitric acid and alcohol there-to, and thereafter separating the desired aliphatic nitrate from the reaction mixture so produced by a process involving extraction of the reaction mixture with a solvent for said aliphatic nitrate and subsequent distillation of the extracted organic constituents of the reaction mixture to separate solvent and alcohol therefrom and returning to the reaction zone alcohol recovered in said distillation step.

25 11. The process of preparing an aliphatic nitrate which comprises continuously passing nitric acid and an aliphatic alcohol together through a reaction zone, continuously removing the reaction mixture from said reaction zone  
30 during the feed of nitric acid and alcohol thereto, and thereafter separating the desired aliphatic nitrate from the reaction mixture so produced by a process involving extraction of the reaction mixture with a solvent for said aliphatic nitrate and subsequent distillation of the extracted organic constituents of the reaction mixture to separate solvent and alcohol therefrom and returning to the solvent extraction step of the process solvent recovered in said distillation step.

12. The process of preparing an aliphatic nitrate which comprises continuously passing nitric acid and an aliphatic alcohol together through a reaction zone, continuously removing the reaction mixture from said reaction zone at approximately the rate of feed of reactants to said reaction zone during the feed of nitric acid and alcohol thereto, and thereafter separating the desired aliphatic nitrate from the reaction mixture so produced by solvent extraction.

13. The process of preparing an aliphatic nitrate which comprises continuously passing nitric acid and an aliphatic alcohol together through a reaction zone, continuously removing the reaction mixture from said reaction zone during the feed of nitric acid and alcohol thereto, and thereafter separating the desired aliphatic nitrate from the reaction mixture so produced by solvent extraction, the amount and concentration of acid continuously introduced into the reaction zone being so co-related to the rate of withdrawal of reactants from said zone as to maintain the degree of concentration of acid in said zone substantially constant.

65 14. The process of preparing an aliphatic nitrate which comprises continuously passing nitric acid and an aliphatic alcohol containing between three and eight carbon atoms inclusive in its aliphatic radical together through a reaction zone, continuously removing the reaction mixture from said reaction zone during the feed of nitric acid and alcohol thereto, and thereafter separating the desired aliphatic nitrate from the reaction mixture so produced by solvent extraction.

15. The process of preparing an aliphatic nitrate which comprises continuously passing nitric acid and an aliphatic alcohol containing between three and eight carbon atoms in its aliphatic radical together through a reaction zone, continuously removing the reaction mixture from said reaction zone during the feed of nitric acid and alcohol thereto, and thereafter separating the desired aliphatic nitrate from the reaction mixture so produced by a process involving extraction of the reaction mixture with a solvent for said aliphatic nitrate, washing with water the material dissolved in the extraction solvent and subsequent distillation of the extracted organic constituents of the reaction mixture to separate solvent and alcohol therefrom.

16. The process of preparing amyl nitrate, which comprises continuously passing nitric acid and amyl alcohol together through a reaction zone, continuously removing the reaction mixture from said reaction zone during the feed of nitric acid and amyl alcohol thereto, and thereafter separating the desired amyl nitrate from the reaction mixture so produced by solvent extraction.

17. The process of preparing amyl nitrate, which comprises continuously passing nitric acid and amyl alcohol together through a reaction zone, continuously removing the reaction mixture from said reaction zone during the feed of nitric acid and amyl alcohol thereto, and thereafter separating the desired amyl nitrate from the reaction mixture so produced by a process

involving extraction of the reaction mixture with a solvent for said amyl nitrate, washing with water the material dissolved in the extraction solvent and subsequent distillation of the extracted organic constituents of the reaction mixture to separate solvent and amyl alcohol therefrom.

18. The process of preparing an aliphatic nitrate which comprises continuously passing nitric acid and a monohydric aliphatic alcohol containing between three and eight carbon atoms inclusive in its aliphatic radical together through a reaction zone, continuously removing the reaction mixture from said reaction zone during the feed of nitric acid and alcohol thereto, and thereafter separating the desired aliphatic nitrate from the reaction mixture so produced by solvent extraction.

19. A process as defined in claim 18, in which 20 the extraction of the aliphatic nitrate from the reaction mixture is accomplished by treatment with a solvent chosen from the class consisting of chlorinated hydrocarbons, benzene, toluene, hexane, heptane and ether.

20. The process of extracting an aliphatic nitrate from a mixture containing said aliphatic nitrate, water, urea, nitric acid, and an aliphatic alcohol which comprises extracting said reaction mixture with a solvent chosen from the class consisting of chlorinated hydrocarbons, benzene, toluene, hexane, heptane and ether.

JOHN F. OLIN.